

# United States Patent

[11] 3,627,594

[72] Inventors **Takaaki Yamamoto;**  
Kaneo Akanuma; Osamu Tanaka, all of  
Kitakyushu, Japan

[21] Appl. No. **781,963**

[22] Filed **Dec. 6, 1968**

[45] Patented **Dec. 14, 1971**

[73] Assignee **Yawata Iron & Steel Co., Ltd.**  
Tokyo, Japan

[32] Priority **Dec. 12, 1967**

[33] **Japan**

[31] **42/79243**

[56]

## References Cited

### UNITED STATES PATENTS

|           |         |                       |             |
|-----------|---------|-----------------------|-------------|
| 2,746,888 | 5/1956  | Ross .....            | 117/221     |
| 2,906,645 | 9/1959  | Carpenter et al. .... | 117/135.1 X |
| 3,058,841 | 10/1962 | Drosten et al. ....   | 117/221 X   |
| 3,151,000 | 9/1964  | Schmidt et al. ....   | 148/113 X   |
| 3,389,006 | 6/1968  | Kohler.....           | 148/113 X   |

*Primary Examiner*—Ralph S. Kendall

*Assistant Examiner*—Caleb Weston

*Attorney*—Wenderoth, Lind & Ponack

[54] **METHOD OF FORMING ELECTRIC INSULATING  
FILMS ON ORIENTED SILICON STEEL**  
7 Claims, No Drawings

[52] U.S. Cl. .... **148/113,**  
148/31.55, 148/6.3

[51] Int. Cl. .... **H01f 1/04**

[50] Field of Search. .... **148/6.3,**  
6.35, 113; 117/135.1, 221

**ABSTRACT:** A method for producing a glassy film having an excellent insulating property on an oriented cold-rolled steel sheet by coating the surface of said silicon steel sheet with a mixture of a Ti compound and an Mg compound and possibly with the addition of an Mn compound thereto and then subjecting the coated silicon steel sheet to a heat-treatment.

**METHOD OF FORMING ELECTRIC INSULATING FILMS  
ON ORIENTED SILICON STEEL**

This invention relates to a method for improving the brittleness of an oriented cold-rolled silicon steel sheet and at the same time forming an electrical insulating film having an excellent electric insulation, adhesion, bendability, space factor and heat resistance on the surface of the oriented cold-rolled silicon steel sheet. The term "oriented cold-rolled silicon steel sheet" used in the present invention means a cold-rolled silicon steel sheet consisting of 2 to 3.5% by weight Si, the rest being Fe and unavoidable impurities, and having a highly oriented crystal grain structure after being finally annealed. Further, it contains in addition one or more of the materials Al (0.1 to 0.09% by weight sol. Al), sulfide, nitride of Mn and V and selenium compound, in small amounts as an inhibitor in order to effect a highly oriented secondary recrystallization during the final annealing. The expression "oriented" means that a great part of crystal grains have (110) [001] crystal orientation, which is called "cube on edge" or (100) [001] crystal orientation, which is called "cube on face."

Oriented cold-rolled silicon steel sheet is used for laminated iron cores or wound iron cores. Such individual silicon steel sheets are coated with electrical insulating films so as to be electrically insulated from each other.

Such electrical insulating film is required to be so tightly adhered to the sheet that it will not be peeled off during working and to have a high space factor and excellent resistance to heat. On the other hand, such insulating film should have no bad influence on the magnetic property of the steel sheet. The silicon steel sheet is generally subjected to a final annealing in which it is treated at a high temperature of about 1200° C. for a long time.

Such final annealing is carried out on steel sheets which are laminated or wound in coils. In such case, in order to prevent the steel plates from sticking to each other due to heat, an annealing separator is used.

For such annealing separator there is utilized a substance which acts to prevent sticking of the steel sheet and at the same time forms a glassy electrical insulating film by reacting with an oxide on the surface of the steel sheet at the annealing temperature.

Substances used for such separators and methods for producing glasslike electrical insulating film are known from U.S. Pat. Nos. 2,354,123, 2,385,332, 2,492,682 and 2,533,351.

These known separators are provided not only for separating action performances but also to form electrical insulating films. Therefore, various film characteristic improving steps can be taken.

For example, there is known a process wherein, during a decarburizing annealing, when Si is selectively oxidized to form  $\text{SiO}_2$  on the steel sheet surface, the steel sheet surface is coated with a suspension consisting of  $\text{MgO}$ ,  $\text{Mg(OH)}_2$  and  $\text{H}_2\text{O}$  and is dried and the steel sheet is then final-annealed at a high temperature in a reducing atmosphere, the  $\text{MgO}$  will act as annealing separators to prevent the steel sheets from sticking to each other and at the same time a part of the materials will react with the above-mentioned  $\text{SiO}_2$  to form a glassy electrical insulating film.

However,  $\text{MgO}$  used as the substance to act as a separator and as a glassy film forming agent. When it is to be applied to a steel sheet, it is generally mixed with water so that it is in the form of a liquid suspension or slurry.

Therefore, there is a disadvantage, that  $\text{MgO}$  acts with water to become  $\text{Mg(OH)}_2$ , which discharges water of hydration while being heated and oxidizes and embrittles the steel sheet.

Such embrittlement causes considerable trouble during the operation of cutting, perforating or winding steel sheets.

As a result of various research made with a view to eliminating the above-mentioned disadvantage and further to reduce the brittleness of steel sheets, the inventors have found that, when a Ti compound such as an oxide or hydroxide of Ti and

an excellent stable and strongly adherent glassy electrical insulating film can be formed on an oriented cold-rolled silicon steel sheet and at the same time the brittleness of said steel sheet can be reduced.

5 An object of the present invention is to provide an insulating film forming process for stably forming a film having an excellent electric insulation property and heat resistance and which is strongly adherent and at the same time reducing the brittleness of the oriented cold-rolled silicon steel sheet itself.

10 It is known that, in order to form an adhesive insulating film,  $\text{SiO}_2$  can be formed on the surface of a silicon steel sheet by selective oxidization so as to be a silicious base for the latter formation of a glassy film. Such a base is formed generally at the time of decarburizing annealing. However, in general, the base composition is so sensitive to the temperature, time, atmosphere and dew point of the atmosphere that it is difficult to obtain a high quality glassy film in a stable manner with known substances capable of serving both as a separator to prevent sticking and as a glassy film forming agent with the result that a film which is poorly adherent is often produced.

15 Particularly, when carrying out a treatment for forming the above-mentioned silicious base layer, when Al in an amount of 0.01 to 0.09 percent by weight sol. Al is contained in the silicon steel sheet as an inhibitor, the Al will also be partly oxidized to produce  $\text{Al}_2\text{O}_3$  which conjointly with the treating conditions influence on the formation of a uniform glassy film, such as impairing the stability of the glassy film and making it more difficult to form a film with excellent electric insulation

20 characteristics, appearance and adhesion.

25 Further, the water contained in the above-mentioned substance will be discharged in the final annealing, which will improperly oxidize the steel sheet and prevent the formation of a high quality glassy film at a temperature particularly above

30 1000° C.

35 The present invention comprises heat-treating for a short time an oriented silicon steel sheet cold-rolled to any desired dimensions, for example in an atmosphere containing wet hydrogen gas so that a surface layer containing  $\text{SiO}_2$  from the selective oxidation of Si in the steel sheet will be selectively formed on the surface of the steel sheet, then coating it with a substance which consists of a mixture of an oxide or hydroxide of Mg such as  $\text{MgO}$  or  $\text{Mg(OH)}_2$  or an oxide or hydroxide such as  $\text{TiO}_2$ ,  $\text{TiO}_2\text{H}_2\text{O}$ ,  $\text{TiO(OH)}_2$  or  $\text{Ti(OH)}_4$  and further heat-treating it in an atmosphere containing hydrogen so that a glassy insulating film will be formed.

40 According to the method of the present invention, a uniform glassy film which is strongly adherent is stably obtained without being influenced by the heat-treating conditions of the atmosphere and the like. Further, the brittleness of the steel sheet itself is greatly reduced.

45 The method of the present invention shall be explained more particularly in the following.

50 As mentioned above the present invention is to be applied to oriented cold-rolled silicon steel sheets. Such an oriented cold-rolled silicon steel sheet is annealed continuously for a short time under a condition, for example, in a wet reducing atmosphere which prevents the oxidization of iron as much as possible but allows the oxidation of silicon in the steel so that  $\text{SiO}_2$  will be formed on the surface of the steel sheet.

55 The heat-treatment for the formation of the above-mentioned  $\text{SiO}_2$  is carried out under a condition which will prevent the oxidization of iron. However, a slight oxidization of iron is not always detrimental. But excess oxidization will reduce the quality of the glassy film and therefore must be avoided.

60 For the heat-treatment for forming  $\text{SiO}_2$  by the selective oxidization on or near the surface of an oriented cold-rolled silicon steel sheet, a reducing atmosphere of hydrogen only or dissociated ammonia is generally used, the dew point of which is 55° to 70° C. and the temperature of which is 700° to 900° C. The longer the treating time, the thicker the oxidized layer and the greater the advantage in the formation of a glassy insulating film. But, the holding time at the above-mentioned temperature is at least one minute or more than one minute.

Needless to say, even when, instead of the short time treatment, a box-annealing is carried out with open coils to form a layer containing  $\text{SiO}_2$  on the surface of the oriented cold-rolled silicon steel sheet, the same favorable result will be obtained. But, in such case, the dew point is preferably below 55° C.

During the above-mentioned heat-treatment for the forming of  $\text{SiO}_2$ , the decarburization of the oriented cold-rolled silicon steel sheet can be simultaneously carried out.

The Mg cold-rolled silicon steel sheet surface on which a layer containing  $\text{SiO}_2$  has been formed is further coated with a substance having as main components one or more mg. compounds such as  $\text{MgO}$  and  $\text{Mg(OH)}_2$  and one or more such Ti compounds such as  $\text{TiO}_2$ ,  $\text{TiO}_3\text{H}_2\text{O}$ ,  $\text{TiO(OH)}_2$  or  $\text{Ti(OH)}_4$ . It is most economical to use this substance as a glassy film-forming agent and also as a material which prevents sticking of the steel sheets during the final annealing.

The above-mentioned substance is formed by mixing 0.5 to 40 parts by weight of a Ti compound with 100 parts by weight of an Mg compound.

When less than 0.5 part of  $\text{TiO}_2$  is used, there will be no effect of the Ti compound and the object of the present invention can not be attained. On the other hand, when more than 40 parts of the Ti compound are used, no high quality glassy film will be obtained. Therefore, 0.5 to 40 parts of the Ti compound are used to make the film agent.

Further, when the amount of the Ti compound is larger than 40 parts, the substance after being dried will be likely to peel off the sheet, during handling the formation of the insulating film will be difficult. A surface having a metallic luster will be exposed and no uniform glassy film will be produced and, even if a phosphate-treatment is thereafter used, no highly adherent film will be obtained.

Further, the Ti compound in the substance has an excellent effect in that it reduces the brittleness of the steel sheet. When 0.5 part of the Ti compound is mixed with 100 parts of the mg. compound, the effect of reducing the brittleness of the steel sheet will appear. When the amount is above the upper limit, there will be no substantial brittleness reducing effect. It is only when 5 to 20 parts of the Ti compound are used that the brittleness will be most reduced.

$\text{MgO}$  which is one of the components of the substance to be used in the present invention may be either a high-temperature baked product or a low-temperature baked product. However, the low-temperature baked  $\text{MgO}$  is more effective for attaining the object of the present invention. Its granularity can be as fine as about 325 meshes to obtain a favorable result.

$\text{TiO}_2$  can be either the rutile type or the anatase type or can be obtained by either low-temperature-dehydrating or high-temperature-baking of metatitanic acid. Its granularity can be fine as about 325 meshes the same as the above-mentioned  $\text{MgO}$  to obtain a favorable result.

The higher the purity of such film substance the better the result. However, even with a reagent of about the first grade or a commercial industrial product, the object of the present invention can be attained.

The film agent substance of the above-mentioned composition is preferably mixed with water so as to form a slurry and the slurry is applied to the surface of an oriented cold-rolled silicon steel on which a layer of  $\text{SiO}_2$  has been formed by selective oxidization. The amount applied is preferably such that the amount of the substance which remains after being dried will be 2 to 10 g./m<sup>2</sup>. When the amount is 4 to 8 g./m<sup>2</sup>., the best result will be obtained.

After the above-mentioned coating, the sheet is dried and is then heated at a high temperature in a reducing atmosphere so that a glassy insulating film will be formed. It is most economical to carry out this glassy insulating film forming treatment at the time of the final annealing of the oriented cold-rolled silicon steel sheet.

That is to say, the oriented cold-rolled silicon steel sheet coated with the above-mentioned substance and then dried is

wound up in the form of a coil or sheets cut to proper dimensions are attacked and final-annealed during which it is held at a high temperature above 1100° C., such as, for example, 1200° C. for more than 5 hours in an annealing furnace in a reducing atmosphere such as, for example, of pure hydrogen.

In such case,  $\text{SiO}_2$  present on the surface of the oriented cold-rolled silicon steel will react with the substance to form a blackish lustrous, compact and rustproof, acidproof high-quality glassy insulating film having a composition in the  $\text{SiO}_2\text{--MgO--TiO}_2$  system.

In the above-mentioned final annealing, the lower the dew point of the atmosphere as the temperature rises, the easier the formation of a high quality film. The substance applied to the surface of the oriented cold-rolled silicon steel sheet is also an annealing separator in the final annealing. That is to say, only a part of the applied substance reacts with  $\text{SiO}_2$  formed on the surface of the steel sheet so as to form a glassy film and the greater part of it remains as an annealing separator on the glassy film formed on the steel sheet surface. Therefore, in order to make the steel sheet into a product, it is necessary to remove the powder by such means as brushing or pickling.

By the above-mentioned treatment according to the present invention, a high-quality insulating film is formed on the surface of an oriented cold-rolled silicon steel sheet and, at the same time, as another feature of the effect of the present invention, the brittleness of the oriented cold-rolled silicon steel sheet itself is reduced. This is presumed to be because the mixture of  $\text{MgO--TiO}_2$  produced during the treatment reacts with

$\text{SiO}_2$  on the surface of the oriented cold-rolled silicon steel sheet to form a compact high quality glassy film, and therefore the oriented cold-rolled silicon steel sheet is not influenced by the annealing atmosphere and the Ti compound acts to directly purify the impurities in the oriented cold-rolled silicon

steel sheet.

Further, in the case of selectively oxidizing an Al-containing oriented cold-rolled silicon steel sheet so that  $\text{SiO}_2$  will be formed on the surface, even when Al is also oxidized to produce  $\text{Al}_2\text{O}_3$ , the above-mentioned substance will be effective. However, the presence of this  $\text{Al}_2\text{O}_3$  will make it difficult to obtain a uniform glassy film and, with the slightest fluctuation of the treating conditions, the formation of the glassy film will be influenced so as to be unstable and a film which is poorly adherent will be likely to be produced.

Therefore, by carrying various experiments to solve the above-mentioned problems, the inventors have discovered that, using the same treatment as is described above by adding to the substance which is the mixture of a Mg compound and a Ti compound a Mn compound in the form of an oxide or a hydroxide, such as  $\text{MnO}_2$ ,  $\text{Mn}_2\text{O}_3$ ,  $\text{Mn(OH)}_2$  or  $\text{MnO-OH}$  or  $\text{MnCO}_3$  which becomes  $\text{MnO}$  when heated, a uniform lustrous glassy film which is strongly adherent can be stably formed on the surface of an oriented cold-rolled silicon steel sheet.

In the substance consisting of the Mg compound, Ti compound and Mn compound, the Mn compound is considered to act to suppress the influence of the  $\text{Al}_2\text{O}_3$  formed on the steel sheet surface. That is to say, when heated, the Mn compound will become  $\text{MnO}$ , will be further reduced by the atmosphere and will enter the steel. The reaction in such case is considered to effectively act on the formation of a film. Further, the oxygen produced by the decomposition of the Mn compound in the reducing atmosphere below 1000° C. is also considered to effectively act.  $\text{MnO}_2$  is excellent in that it is a compound which discharges oxygen and is readily available. Its granularity should be about 325 meshes to obtain favorable results.

In an experiment, when an oriented cold-rolled silicon steel sheet produced from a hot-rolled silicon steel sheet containing 0.030 percent sol. Al was coated with a substance within the scope of the present invention, was then heat-treated and was taken out and the substance was analyzed, the content of  $\text{Al}_2\text{O}_3$  was 1.1 to 21.1 percent.

The substance effective for application to the above-mentioned Al-containing oriented cold-rolled silicon steel sheet is

formed by mixing 0.5 to 80 parts, preferably 2 to 40 parts of a Ti compound and 0.5 to 50 parts, preferably 2 to 25 parts, of a Mn compound with 100 parts of a Mg compound.

In the above-mentioned composition, when the Ti compound is below the above-mentioned range, no effect of the compound will be obtained and, on the other hand, when it exceeds 80 parts, the substance after being dried will be likely to be peeled off by the slightest contact or shock and the formation of the insulating film will become difficult.

Further, when the Mn compound is below the above-mentioned range, it will not be effective. On the other hand, when it is used in excess of 50 parts, the amount of oxygen discharged during the heat-treatment will be so large that the atmosphere will become oxidative and will have a bad influence on the formation of the glassy insulating film.

The substance of the above composition is not only effective for application particularly to an Al-containing oriented cold-rolled silicon steel sheet but also can be applied to such oriented silicon steel sheet containing no Al as is described above.

The substance of the present invention has been described in detail above. Further, a comparison of the differences in characteristics obtained, when known substances using MgO and the substances of the present invention are used, but the other conditions are exactly the same, will be described with reference to examples in the following.

#### EXAMPLE 1

An oriented cold-rolled steel sheet having 3.25 percent Si and reduced to a final thickness of 0.35 mm. was annealed for a short time of 5 minutes at a temperature of 800°C. in a wet dissociated ammonia atmosphere having a dew point of 61°C. so that  $\text{SiO}_2$  was selectively formed on the steel sheet surface, coated with a substance at each of the mixing rates in table 1 so that the amount coated on the sheet was 6 g./m.<sup>2</sup> and was final-annealed for 20 hours at a temperature of 1200°C. in a dry hydrogen atmosphere. The characteristics of the thus formed glassy insulating films are shown in table 2. The films

30 35 40

TABLE 2.—GLASSY FILM CHARACTERISTICS

| Sample Numbers | Layer resistance <sup>1</sup>           | Properties                                    |  |
|----------------|-----------------------------------------|-----------------------------------------------|--|
|                |                                         | Adhesion after phosphate-coating <sup>2</sup> |  |
| 1              | 4.30 $\Omega\text{-cm.}^2/\text{sheet}$ | Partly peeled off.                            |  |
| 2              | 11.5 $\Omega\text{-cm.}^2/\text{sheet}$ | Not peeled off.                               |  |
| 3              | 19.4 $\Omega\text{-cm.}^2/\text{sheet}$ | Little peeled off.                            |  |
| 4              | 9.28 $\Omega\text{-cm.}^2/\text{sheet}$ | A little peeled off.                          |  |
| 5              | 0.20 $\Omega\text{-cm.}^2/\text{sheet}$ | Almost peeled off.                            |  |

10 15 20 25

<sup>1</sup> (Under 35 kg./cm.<sup>2</sup> by ASTM method 2).  
<sup>2</sup> As bent by 180 degrees to a diameter of 20 mm.

NOTE.—The phosphate coating was obtained by applying magnesium phosphate onto the glassy film and heating it at 800°C. for 30 seconds in  $\text{N}_2$  gas. The amount of coating on the film was 3 g./m.<sup>2</sup>.

15 20 25

TABLE 3.—BRITTLENESS OF STEEL SHEETS ON WHICH GLASSY FILMS WERE FORMED

| Sample Number | Characteristics—bending frequency (by ASTM method) |             |             |           |
|---------------|----------------------------------------------------|-------------|-------------|-----------|
|               | <10 times                                          | 11-20 times | 21-30 times | >31 times |
| 1             | 20                                                 | 2           | 6           | 12        |
| 2             | 0                                                  | 7           | 16          | 17        |
| 3             | 2                                                  | 24          | 11          | 2         |
| 4             | 1                                                  | 19          | 16          | 13        |
| 5             | 17                                                 | 3           | 0           | 0         |

#### EXAMPLE 2

An oriented cold-rolled steel sheet of 0.032% total Al and 2.9% Si and reduced to a final thickness of 0.30 mm. was continuously annealed for a short time of 4 minutes at a temperature of 850°C. in a wet dissociated ammonia atmosphere having a dew point of 65°C. so that  $\text{SiO}_2$  was selectively formed on the surface, was then coated on the surface with a substance at each of the mixing rates and with the compositions shown in table 4 so that the amount of the substance remaining after being dried was 5.5 g./m.<sup>2</sup>, was dried and was then final-annealed for 15 hours at a temperature of 1200°C. in a dry hydrogen atmosphere so that a glassy film was formed.

40

TABLE 4.—COMPOSITIONS OF SUBSTANCES

| Sample number | Composition |                          |                          |                                           |
|---------------|-------------|--------------------------|--------------------------|-------------------------------------------|
|               | MgO, grams  | TiO <sub>2</sub> , grams | MnO <sub>2</sub> , grams | Water, liters                             |
| 1             | 100         | 0                        | 0                        | 1 Control.                                |
| 2             | 100         | 0                        | 25                       | 1 Do.                                     |
| 3             | 100         | 20                       | 0                        | 1 Substance (A) of the present invention. |
| 4             | 100         | 20                       | 6                        | 1 Substance (B) of the present invention. |
| 5             | 100         | 20                       | 13                       | 1 Do.                                     |
| 6             | 100         | 27                       | 7                        | 1 Do.                                     |
| 7             | 100         | 30                       | 14                       | 1 Do.                                     |
| 8             | 100         | 36                       | 7                        | 1 Do.                                     |
| 9             | 100         | 40                       | 15                       | 1 Do.                                     |
| 10            | 100         | 20                       | 6                        | 1 $\text{SiO}_2$ was not formed.          |

made by the method of the present invention are more compact and much more strongly adherent than by the known processes.

Further, in table 3 there are shown the results of bending tests by the ASTM method to show the effects of reducing the brittleness of the steel sheets after the formation of glassy films. It is clear that the brittleness is greatly reduced in the films made by the method of the present invention.

TABLE 1.—COMPOSITIONS OF USED FILM AGENTS

| Sample Number | Composition |                          |                                                    |
|---------------|-------------|--------------------------|----------------------------------------------------|
|               | MgO, grams  | TiO <sub>2</sub> , grams | Water, liters                                      |
| 1             | 100         | 0                        | 1 Control.                                         |
| 2             | 100         | 10                       | 1 Film agent (A) adopted in the present invention. |
| 3             | 100         | 25                       | 1 Do.                                              |
| 4             | 100         | 40                       | 1 Do.                                              |
| 5             | 100         | 100                      | 1 Control ( $\text{SiO}_2$ was not formed).        |

60 65 70 75

TABLE 5.—GLASSY FILM CHARACTERISTICS

| Sample Number | Layer resistance <sup>1</sup>           | Characteristics                               |  |
|---------------|-----------------------------------------|-----------------------------------------------|--|
|               |                                         | Adhesion after phosphate-coating <sup>2</sup> |  |
| 1             | 0.49 $\Omega\text{-cm.}^2/\text{sheet}$ | Pealed off.                                   |  |
| 2             | 0.91 $\Omega\text{-cm.}^2/\text{sheet}$ | Partly peeled off.                            |  |
| 3             | 6.15 $\Omega\text{-cm.}^2/\text{sheet}$ | A little peeled off.                          |  |
| 4             | 10.5 $\Omega\text{-cm.}^2/\text{sheet}$ | Do.                                           |  |
| 5             | 15.8 $\Omega\text{-cm.}^2/\text{sheet}$ | Almost peeled off.                            |  |
| 6             | 15.1 $\Omega\text{-cm.}^2/\text{sheet}$ | A little peeled off.                          |  |
| 7             | 24.3 $\Omega\text{-cm.}^2/\text{sheet}$ | Little peeled off.                            |  |
| 8             | 20.4 $\Omega\text{-cm.}^2/\text{sheet}$ | Do.                                           |  |
| 9             | 18.4 $\Omega\text{-cm.}^2/\text{sheet}$ | Do.                                           |  |
| 10            | 0.13 $\Omega\text{-cm.}^2/\text{sheet}$ | Little peeled off.                            |  |

<sup>1</sup> (Under 35 kg./cm.<sup>2</sup> by ASTM method 2).  
<sup>2</sup> As bent by 180 degree to a diameter of 20 mm.

#### EXAMPLE 3

An oriented cold-rolled silicon steel having 0.03 percent total Al and 2.85% Si was rolled to a sheet 0.15 mm. thick, was continuously annealed for a short time of 4 minutes at a temperature of 850°C. in a wet decomposed atmosphere hav-

ing a dew point of 65° C. so that  $\text{SiO}_2$  was selectively formed on the surface, was coated on the surface with a substance at each of the below-mentioned mixing rates so that the amount of the substance after drying would be 6 g./m.<sup>2</sup>, was dried and was then final-annealed for 20 hours at a temperature of 1200° C. in a dry hydrogen atmosphere so that a glassy film was formed. As a result, excellent electrical insulating films as described below were obtained.

| Composition |       |                          | Layer <sup>1</sup><br>resist-<br>tance | Surface appearance<br>after removing powder  |
|-------------|-------|--------------------------|----------------------------------------|----------------------------------------------|
| MgO         | TiO   | $\text{MnO}_2$ ,<br>gram |                                        |                                              |
| 100 percent |       |                          | 0.41                                   | No glassy film was produced.                 |
| 20 grams    | Large | 0.6                      | 3.95                                   | A uniform lustrous glassy film was produced. |

<sup>1</sup> After removing powder in  $\Omega\text{-cm.}^2/\text{sheet}$  (under 35  $\text{kg./cm.}^2$ ).

What is claimed is:

1. A method for producing an electrical insulation film on an oriented silicon steel sheet containing 0.01 to 0.09 wt. percent sol. al. comprising the steps of subjecting the silicon steel sheet to a heat-treatment at a temperature of 700° to 900° C. to form  $\text{SiO}_2$  on the surface of the steel sheet, applying to the said surface of the steel sheet a slurry by mixing (1) 0.5 to 80 parts by weight of at least one compound selected from the group consisting of an oxide of Ti and a hydroxide of Ti, (2) 0.5 to 50 parts by weight of at least one compound selected from the group consisting of an oxide of Mn and a hydroxide of Mn, and (3) 100 parts by weight of a compound selected from the groups consisting of an oxide of mg. and a hydroxide

of mg. drying the steel sheet coated with the slurry, and annealing the said steel sheet in a hydrogen-containing atmosphere at a temperature above 1100° C.

2. The method claimed in claim 1, wherein the oriented cold-rolled silicon steel sheet contains 2 to 3.5 wt. percent Si.

3. The method claimed in claim 1 wherein the heat-treatment for forming  $\text{SiO}_2$  on the surface of the steel sheet comprises holding said steel sheet at a temperature of 700° to 900° C. for at least 1 minute in a reducing atmosphere of hydrogen

10 only.

4. The method claimed in claim 1, wherein the heat-treatment for forming  $\text{SiO}_2$ , on the surface of the steel sheet comprises holding said steel sheet at a temperature of 700° to 900° C. for at least 1 minute in a reducing atmosphere containing 15 dissociated ammonia and having a dew point of 55° to 70° C.

5. The method claimed in claim 1, wherein the slurry is prepared by mixing the mixture with water and is applied on the surface of the oriented silicon steel sheet on which  $\text{SiO}_2$  has been formed in an amount such that the amount of the

20 deposited material left after it has been dried is 2 to 10 g./m.<sup>2</sup>.

6. The method claimed in claim 1, wherein the slurry is prepared by mixing (1) 2 to 40 parts by weight of a compound selected from the group consisting of an oxide of Ti and a hydroxide of Ti, (2) 2 to 25 parts by weight of a compound selected from the group consisting of an oxide of Mn and a hydroxide of Mn and (3) 100 parts by weight of a compound selected from the group consisting of an oxide of Mg and a hydroxide of Mg.

7. The method claimed in claim 6 wherein only one compound from each group is mixed in said slurry.

\* \* \* \* \*

35

40

45

50

55

60

65

70

75